

Nov. 4, 1924.

1,514,335

G. H. PHELPS ET AL

PRESS FORGING AND SIMILAR OPERATION

Filed Dec. 15, 1921

Fig. 1,



Fig. 2,



Fig. 3,



Fig. 6,



Fig. 7,



Fig. 4,



Fig. 5,



## UNITED STATES PATENT OFFICE.

GEORGE H. PHELPS, OF WAREHOUSE POINT, CONNECTICUT, AND THOMAS E. MURRAY, JR., OF BROOKLYN, NEW YORK; SAID PHELPS ASSIGNOR TO THOMAS E. MURRAY, OF BROOKLYN, NEW YORK.

## PRESS FORGING AND SIMILAR OPERATION.

Application filed December 15, 1921. Serial No. 522,480.

To all whom it may concern:

Be it known that we, GEORGE H. PHELPS and THOMAS E. MURRAY, Jr., citizens of the United States, said PHELPS residing in 5 Warehouse Point, Connecticut, and said MURRAY residing in Brooklyn, New York, have invented certain new and useful Improvements in Press Forgings and Similar Operations, of which the following is a 10 specification.

The present invention provides a method and apparatus by which metal or metals can be worked and shaped economically and expeditiously to secure products which are 15 now made by press forging, die casting, extruding and similar operations in which the metal is softened or melted and shaped by means of molds, dies or the like.

The accompanying drawings illustrate 20 embodiments of the invention.

Fig. 1 illustrates in section the parts in their initial position;

Fig. 2 is a similar section of the finished 25 forging;

Fig. 3 is a plan of a portion thereof;

Fig. 4 is a section similar to Fig. 1 illustrating an alternative method;

Fig. 5 is a plan on the line 5—5 of 30 Fig. 4;

Figs. 6 and 7 are sections of other alternatives.

Referring to Figs. 1, 2 and 3, the forging to be made is a gear blank 1 of aluminum or other soft metal with a reinforcing disc 25 2 of steel or other comparatively strong metal embedded in the aluminum.

The metal in the beginning is in the form 40 of rods 3, 4 (Fig. 1) of aluminum with a plate 5 of steel (which in the instance shown is to be unchanged in shape in the final product, but which in other cases may be shaped by the forging operation). These pieces 3, 4 and 5 are introduced as shown into a tubular mold 6 at the lower end of 45 which is a terminal 7 of copper mounted on a support 8. The terminal 7 is insulated from the casing 6 and in the upper end of the latter there is a movable terminal 9 bearing on top of the slug 3. The terminals 50 7 and 9 are at the opposite ends of an electric circuit and when the current is applied it passes through the pieces of metal 3, 5 and 4 to soften them; and the upper terminal 9 is pressed downward to forge the

mass of metal into the desired shape. The 55 ends of the terminals 7 and 9 are shaped to produce the desired configuration on the top and bottom of the forging. A slight membrane or fin, 1<sup>a</sup>, left in the center may be easily punched out afterwards. 60

The mold 6 may be of various materials, such, for example, as chilled cast steel. The terminals 7 and 9 may be steel or copper inserts constituting the ends of electrodes. The lower terminal may be held stationary, 65 being in that case in effect a fixed part of the mold, while the upper one constitutes the plunger, moved downward as indicated by the arrow by means of any suitable motor. A solenoid designed so as to give 70 any desirable rate of movement of the metal may, for example, be used as the motor.

In the arrangement shown in Figs. 4 and 5 the two electrode terminals 10 and 11 are stationary and located at opposite ends of 75 the mold 12 which is insulated from the lower terminal. The metal to be forged is in the form of a cylindrical blank or slug 13 and, when sufficiently heated by the passage of the current, is forged by the downward movement of a presser 14 which forms a socket in the top of the blank and presses the metal out at the sides into the annular recess 15. Such a mold would have to be split as shown in Fig. 5 to permit removal 80 of the forging; the two parts being guided in their movement toward and away from each other on guide rods 16. An annular space 17 or clearance should be left between the sides of the mold and the blank 13 so 85 that current will pass through the latter and not through the mold itself. 90

Fig. 6 shows another arrangement for producing the product of Fig. 2, in which the recesses constituting the hole in the 95 center of the product are made by means of plungers 18 and 19 passing through the electrode terminals 7 and 9. Here we have shown the metal to be forged in blanks of slightly different design from those of Fig. 1; a single rod 20 of aluminum extending between the terminals and passing through a ring 21 of steel. In operation the plungers will move inward to the desired positions with relation to the terminals, after which 100 the upper terminal and the plunger 18 will move down together to the final position. 105 This arrangement gives better contact

surfaces between the blank 20 and the electrodes and reduces the heating effect on the electrodes at their point of contact with the blank.

5 It is not essential that the mold be a closed one. In Fig. 5, for example, the two halves of the mold 12 may be separated in the beginning and may be brought together to compress the product simultaneously with 10 or immediately after the passing of the current.

In Fig. 7 we have shown an arrangement of the same character for producing the product of Fig. 2. The terminals 7 and 9 15 and the plungers 18 and 19 are the same as in Fig. 6. The sides of the mold, however, are formed by flanges 22 and 23 projecting inward from the heads of the terminals and constituting in fact parts of the same. In 20 this case, as in the described use of the split mold of Fig. 5, the metal to be forged in the beginning is confined between the terminals constituting parts of the mold; but the heating operation is initiated while the 25 metal is actually in the open air, and the mold is not closed until the parts are brought together as described.

In operation a pressure will be put upon the plungers and the electrodes so that as 30 soon as the current is applied the plungers will move inward and the terminal 9 will move downward until its flange 22 engages the flange 23 of the lower terminal, thus enclosing the product, with a small fin between the flanges, which can be easily removed afterwards.

Various other styles of mold and other arrangements of the electrode terminals and 40 pressers may be utilized in carrying out the invention.

In a patent of Thomas E. Murray, Jr., No. 1,281,636, of October 15, 1918, there is described a method of electric welding which consists in subjecting the parts to 45 be united to a current of extremely high ampere strength or current density per square inch, and of very brief duration. We prefer to apply the current in the same way to the present forging operation. For 50 example, we may utilize a current of ninety thousand amperes or more per square inch applied for about a quarter of a second in the case of small forgings. This, however, is not the only method of heating with the 55 electric current within our invention. The shaping of the product by a very quick operation may be accomplished with other methods of application of the current.

The quick upsetting of the metal and the 60 necessary pressure for obtaining such a quick operation serve to produce considerable heat in addition to that produced by the passage of electric current.

65 Preferably also the entire blank is confined within the mold and is engaged by the

presser at a point within the mold. By using an electrode terminal which shapes the portion of the blank which it engages the construction of the mold is simplified for many forgings. Various other means 70 and methods, however, may be used for forcing the metal under pressure into the shape of the mold.

By our improved method the operation is so quick as to practically avoid oxidation, 75 and the confinement of the blank within the mold aids in securing this result. Likewise the speed of the operation is such that there is practically no loss of heat by radiation. The greatest advantage of the 80 invention lies in the uniformity with which a number of such operations can be performed. The current can be controlled as to intensity and duration with great accuracy, and so can the take-up or movement 85 of the presser. Thus we will have a uniform heating over a uniform period of time, a uniform speed of operation or flow of the metal and a uniform density of the resulting forging. The current will be continued 90 only long enough to bring the metal to the exact degree of plasticity required for the particular molding operation, producing an actual liquefaction or even a vaporization 95 thereof if that should be necessary for fine and intricate forging. The pressure will generally be applied before the closing of the electric circuit so as to take effect as soon as the metal softens and will, of course, be continued throughout the take-up of the 100 presser. Generally the current will be broken before the completion of the take-up so that the actual forging and densifying operations will continue while the metal is cooling from its maximum temperature.

105 While we have referred to the operation as "press forging," it may be applied in such a way as to be practically a die casting operation in which liquid metal is forced into a die and cooled therein under pressure. A sufficient current may be used to liquefy the metal, or even to vaporize it if necessary, so as to permit the forcing of it 110 into the sharpest corners and the most intricate shapes. Ordinary die casting operations are limited to certain metals which can be maintained at the desired fluidity while being transferred into the die. With the present invention metals can be die cast which are not susceptible to such treatment 115 by the old method; the present invention being practically without limit in this respect.

120 The process in some cases may be made to partake of the nature of an extruding operation in part or in whole. For example, it may be said, in comparing Figs. 1 and 2, that a portion of the aluminum rods 3 and 4 is extruded through the center of the steel ring 3. The process presents such wide 125

possibilities in the matter of temperature control that it may in fact be applied to operations in which the metal to be worked is partly forged, partly cast and partly extruded to secure a product of the desired shape. The process is applicable also not only to the reshaping of the entire blank but to the reshaping of only one end or other part of the blank, as in the upsetting 10 of a bolt head or a more complicated shape on the end of a rod.

In fact, where the metal is rendered sufficiently fluid we may, for some products, do without any special pressing mechanism, 15 relying on the weight only of the upper electrode to maintain it in contact with the work during the operation.

An important feature of the invention is its applicability to the making of products 20 composed of two or more metals of different melting points, such as the aluminum and steel product of Figs. 2 and 3. In working with a plurality of metals the temperature may be regulated to such a point as to fuse 25 one of the metals and not the other or others, or even to volatilize one or more of them, or merely to soften them sufficiently for the particular purpose in hand.

We have referred to steel and copper as 30 examples of suitable metals for the terminals but there are various other metals or alloys or compositions having suitable electrical and physical properties to permit their use instead of steel and copper. It is important, 35 though not always essential, that the blank be of less cross-section than the terminal from which it receives its current. Thus the total conductivity of the terminal will be greater than that of the blank and the heating effect on it will be less in the cases illustrated. In the cases illustrated a blank of comparatively small cross-section is used 40 with comparatively large terminals. Consequently, in order to provide sufficient metal 45 to make the product of the full width of the terminals the blank has to take a long shape for such products as are illustrated. For other cases, however, the length, in proportion to the diameter may, of course be less. 50 This means a very considerable working of the metal, which is advantageous. It also allows a long stroke of the machine producing a high pressure on the product at the end of the stroke.

55 Though we have described with great particularity of detail certain embodiments of our invention yet it is not to be understood therefrom that the invention is restricted to the particular embodiments disclosed. Various 60 modifications thereof may be made by those skilled in the art without departure

from the invention as defined in the following claims.

What we claim is—

1. In press forging and similar operations 65 using a mold, the method which consists in heating the metal to be forged by the passage of an electric current through a circuit including such metal and a part of the molding surface and pressing the metal into the 70 shape of the mold by means engaging the metal at a point within the mold.

2. In press forging and similar operations, the described method which consists in heating the metal to be forged by subjecting it 75 to a current of extremely high ampere strength and of very brief duration and pressing it into a desired shape while thus heated.

3. In press forging and similar operations 80 the method which consists in heating the metal while in a mold by the passage through it and through a part of the molding surface of an electric current to a sufficient temperature and pressing it into the shape of the 85 mold, the heating and shaping of the metal being effected in a very brief interval of time.

4. In press forging and similar operations using a mold, the method which consists in heating the metal to be forged by the passage 90 of an electric current through a circuit including such metal and a part of the molding surface, while the metal is entirely confined within the mold.

5. In press forging and similar operation, 95 the method which consists in heating the metal to be forged within a mold by subjecting it to a current of extremely high ampere strength and of very brief duration and pressing it into the shape of the mold while 100 thus heated.

6. An apparatus for press forging and the like, including in combination a mold adapted to enclose the entire body of metal 105 to be forged and means for heating such metal including a terminal constituting part of the molding surface, and means for pressing the metal into the shape of the mold.

7. An apparatus for press forging and the like, including in combination a mold adapted to enclose the entire body of metal to be forged and means for passing an electric current through such metal including a terminal constituting part of the molding surface, and means for pressing the metal heated by such current into the shape 110 of the mold.

In witness whereof, we have hereunto signed our names.

GEORGE H. PHELPS.  
THOMAS E. MURRAY, JR.